

G. E. WEISSENBURGER.  
PROCESS FOR MAKING STEEL.  
APPLICATION FILED FEB. 29, 1912.

1,140,550.

Patented May 25, 1915.



Fig. 1.



Fig. 2.

Witnesses:

Robert H. Weis  
Charles A. Seem

Inventor:  
George E. Weissenburger  
By Brown & Hopkins Atty's

# UNITED STATES PATENT OFFICE.

GEORGE E. WEISSENBURGER, OF BERLIN, GERMANY, ASSIGNOR OF ONE-HALF TO OTIS ELEVATOR COMPANY, OF NEW YORK, N. Y., A CORPORATION OF NEW JERSEY.

## PROCESS FOR MAKING STEEL.

1,140,550.

Specification of Letters Patent. Patented May 25, 1915.

Application filed February 29, 1912. Serial No. 680,766.

*To all whom it may concern:*

Be it known that I, GEORGE E. WEISSENBURGER, a citizen of the United States, residing at Berlin, Germany, have invented certain new and useful Improvements in Processes for Making Steel, of which the following is a full, clear, and exact specification.

The invention relates to an improved process in making steel, and particularly to an improved process and furnace adapted for making steel castings.

The primary object of the invention is to provide an improved process of making steel of the character herein described, and which is adapted to permit the use of a large percentage of steel scrap and pig iron possessing a less quantity of silicon in its composition than has heretofore been found permissible to use in Bessemer converters of either the bottom or side blow type and yet obtain steel sufficiently high in temperature to successfully cast delicate and intricate shapes.

To the attainment of these ends and the accomplishment of other new and useful objects, as will appear, the invention consists in the features of novelty, in the construction, combination and arrangement of the several parts hereinafter more fully described and claimed, and shown in the accompanying drawings, in which—

Figure 1 is a vertical section through the center of the furnace taken at right angles to the axis on which the converter is mounted; Fig. 2 shows a plan view of the forward part of the furnace and a horizontal sectional view of the rear portion.

The furnace may be of the common form or shape and of the tilting type. The walls 40 of the same, indicated by the reference numeral 1, are constructed of material commonly used for such purposes and old and well known in the art. An opening is provided at the top of the furnace through 45 which the metal may be charged into it, and is provided with a suitable covering or door 2, hinged or otherwise secured to the walls of the furnace. A discharge spout 3 is provided for withdrawing the metal after being converted into steel. The sides of the 50 furnace are provided with suitable trunnions firmly secured thereto and forming the axis on which the furnace is pivotally mounted. The trunnions 4 and 5 are rotatably secured in suitable bearings 6 and 7

on the upright supporting members 8 and 9, which may be of any desired form or construction. In the present embodiment the furnace is illustrated as the side blow type, and is provided with the usual set of tuyers 50 10. A suitable pipe or passage 11 communicates with the tuyers 10, and in order that the furnace may be freely rotated this pipe or passage 11 is extended to a line at the side of the furnace coinciding with the extended axis, according to the construction well known in converters of this character. The supply-pipe 11 is provided with a suitable gate valve or other suitable controlling means, and in the present embodiment of the 70 invention is shown as a branch of the pipe or tube 13 which coincides with the extended axis of the furnace and is provided with another branch 14 extending upwardly over the top of the furnace on the side adjacent 75 to the spout 3. This pipe 14 is also provided with a suitable gate valve or control 15. The pipe connects with tuyers 16 which enter the interior of the furnace far above the surface of the metal as illustrated, 80 while the set of tuyers 10 first described are located only slightly above the surface of the metal, so that the air admitted through them will strike the metal. The tuyers 10 may be of any desired number 85 and likewise as many of the tuyers 16 as desired may be employed, although in the present embodiment only two are shown. The tuyers 16 are preferably provided as shown in the embodiment with suitable oil 90 or gas burners 17, one of such burners being adjacent to each of the tuyers, and each of the burners 17 may be fed from a common source of supply, as the feed pipe 18 which leads into the common header or connecting pipe 19. Air to the tuyers 10 is supplied through the pipe 11, and the pipe 14 being also a branch of the pipe 13, receives its supply of air from the same source 95 as the pipe 11, and although this is a convenient construction, it will be apparent that each set of the tuyers 10 and 16 may receive its air supply from independent sources, if desirable. The gas or oil burners 100 17 are each provided with individual controlling means 17a.

Having set forth the construction of a furnace that may be used, its mode of operation in the improved process of making steel will now be described.

It has been found preferable, although not essential, to first heat the furnace by the combustion of oil or gas, admitted through the twyers 16. The metal is then charged into the furnace either in the solid state, or part of it in the solid state and the remainder in the molten state, or, if desired, all of it may be melted before being charged into the furnace. Air and oil, or gas, of the proper proportions and under the most desirable pressure for economic combustion are then admitted through the twyers 16 by means of the gate valve 15 and the burner controlling means 17<sup>a</sup>, until the molten material has reached the temperature where the oxidation of silicon begins to take place. Air is then admitted through the twyers 10 by opening the gate valve 12, and the silicon and manganese in the molten material are rapidly removed by oxidation. If the oxidation of the silicon increases the temperature of the metal to a point where the combustion of carbon takes place, the carbon will be eliminated after the silicon and manganese, and if there is not sufficient silicon in the molten material to raise the temperature to where the combustion of the carbon takes place, the additional temperature required may be supplied by the combustion of fuel admitted through twyers 16. After the combustion of carbon begins it is rapidly removed, after which the molten metal is ready to be re-carbonized and poured into the molds.

Heretofore it has been the practice to reduce the charge of metal in a cupola or melting furnace to a molten condition and then introduce it into a converter; or the molten metal has been transferred directly from a blast furnace into a converter. Converters of the ordinary type are provided with twyers for the admission of air in the form of a blast. When this blast of air is forced into the charge within the converter which necessarily must be rich in silicon, the oxidation of the silicon begins. This oxidation of the silicon raises the temperature of the charge until the temperature reaches a point where the combustion of carbon begins, which further increases the temperature until the carbon is eliminated, after which the metal is ready to be re-carbonized and poured into molds. In the process above described, if there be any manganese in the bath or charge, it will be removed about the same time that the silicon is removed, and will aid the latter in raising the temperature. However, there must be sufficient silicon and manganese in the charge so that the oxidation of these elements will raise the temperature of the charge to a point where the oxidation of the carbon begins, otherwise when the air blast is introduced into the charge in the converter, it will chill the contents before the reduction

of the carbon begins, thus causing a failure in converting the charge.

It is often very much desired to utilize considerable quantities of scrap metal in making the steel, but it has often been found that when considerable quantities of scrap are used in the process described, such scrap causes the amount of silicon in the charge to be lowered to such a point that when the silicon and manganese oxidize, the temperature is not raised sufficiently to cause the oxidation of the carbon and therefore conversion of the charge fails. In order to overcome this difficulty, the converter shown in the drawings is not only provided with twyers for furnishing the air blast but also with twyers for burning oil or gas or other highly inflammable material. Therefore, instead of heating the charge in a cupola, which charge may include large quantities of scrap, it may be introduced directly into the converter, and by the use of the heating twyers, the temperature of the charge may be raised to any desired point before the air blast is turned on, so that regardless of the amount of silicon or manganese, or other easily oxidized elements in the charge, the temperature of the charge may with certainty be brought to a point where the oxidation of the carbon begins. Then the heating twyers may be turned off if desired, and the air blast introduced, and the converting process will proceed until completed, as the carbon having once begun to be oxidized, will continue to oxidize.

Materials such as silicon and manganese when a certain temperature is reached become oxidized, after which they are oxidizing agents with respect to the carbon which is oxidizable because at a still higher temperature the carbon is oxidized. The oxidizable carbon is oxidized more easily the greater the amount of silicon or manganese present because then the heat capable of being produced is greater and the amount of oxidizing agents such as the oxidized silicon and manganese is also greater.

It will therefore be seen that my improved process consists in combining in one continuous operation, the open-hearth process and the Bessemer or converter process; both of these operations are carried on within a single device, namely, the converter into which the air blast is introduced preferably after the heating twyers have been turned on for the requisite length of time. Although the heating twyers may be left turned on after the air blast begins to operate, it is preferred to first heat the charge to the requisite temperature by the heating twyers, and then turn them off again either shortly before or after the blasting twyers are turned on, as it is unnecessary to keep the heating twyers turned on after the air blast is introduced.

In order that the invention might be fully understood, the details of an embodiment have been thus specifically described, but what I claim is:

- 5 A method of making steel which comprises applying heat to a charge of iron low in oxidizable agents within a Bessemer converter until oxidation of the carbon begins, then discontinuing the application of
- 10 heat and directing a blast of air against the charge until substantially all of the oxi-

dizable agents have been eliminated by oxidation.

In testimony whereof I have signed my name to this specification, in the presence of 15 two subscribing witnesses, on this 12th day of February A. D. 1912.

GEORGE E. WEISSENBURGER.

Witnesses:

WOLDEMAR HAUPT,  
HENRY HASPER.